

Feb. 3, 1931.

G. L. SCHWARTZ

1,791,248

## FELTED CELLULOSE FIBER PRODUCT

Filed Sept. 22, 1928



Fig. 2



Fig. 1

GEORGE L. SCHWARTZ: Inventor

By his attorney

Albert T. St. Clair

## UNITED STATES PATENT OFFICE

GEORGE L. SCHWARTZ, OF WILMINGTON, DELAWARE, ASSIGNOR TO E. I. DU PONT DE NEMOURS & COMPANY, OF WILMINGTON, DELAWARE, A CORPORATION OF DELAWARE

## FELTED-CELLULOSE-FIBER PRODUCT

Application filed September 22, 1928. Serial No. 307,760.

This invention relates to the art of cellulose products and more particularly to the art of felted cellulose fiber products.

Many attempts have been made to produce cellulose fiber products by compacting the fibers into a felt but the results achieved by previous processes have been subject to various objections. In the prior processes it has been customary to use binding materials to unite the fibers but this is objectionable because it gives a product of low porosity. On the other hand, when a binding material has not been used in the previous processes, the resulting felt has been inherently weak. Also, the products resulting from previous processes have often been stiff and horn-like, because the gelatinizing action of the substances used for treating the fibers, such as aqueous solutions of caustic soda or zinc chloride, has not been stopped by heat.

It is an object of the present invention to produce felted cellulose fiber products without the use of auxiliary binding materials.

It is another object of the present invention to produce cellulose fiber products having a high degree of pliability.

It is a further object of the present invention to produce these products that they shall have a greatly increased wet strength.

It is a still further object of the present invention to produce such products having an increased dry strength without being susceptible to the customary "paper break".

It is a still further object of the present invention to produce cellulose fiber products having increased wet and dry strength without impairing their wetting properties or reducing their porosity.

With the above and other objects in view, which will be apparent as the description proceeds, I have set forth my invention in the following specification and illustrated it in the accompanying drawing, in which:

Fig. 1 is a diagrammatic side elevation of an apparatus for carrying out my invention, and

Fig. 2 is a diagrammatic plan view thereof.

In the accompanying drawing 10 designates a continuous roll of felt composed of fibers that are curled and kinked and which has

been made in any desired manner. This may be accomplished, for example, as set forth in the copending application of McCormick and Schwartz, Serial No. 283,445, filed June 6, 1928, the process consisting, briefly, in 55 treating cellulose fibers with a solution of caustic alkali for example 8 to 35% sodium hydroxide, at temperatures from slightly below 5° C. to 60° C. This pulp can then be converted into a continuous roll of felt by any 60 standard paper machinery, such as a Fourdrinier machine.

The roll of felt 10, mounted in any desired manner, passes over a guide roll 11 and is fed on to a wire screen conveyor 12, which 65 may be made of any suitable material, such as Monel metal, and is supported by guide rolls 13, 14, 15, 16 and 17, and a drum which will be described hereinafter.

The conveyor 12 propels the felt 10 forwardly into a bath of cold caustic solution 18, which is kept in circulation through an overflow connection 19 between a main caustic tank 20 and an overflow tank 21, and by providing the latter with a gravity outflow pipe 75 22 at a point slightly above its bottom. From this pipe the solution flows into a pump 23, driven by any suitable means, which forces the solution up to a supply tank 24, from which it flows by gravity back to the tank 20. The supply tank 24 may be cooled by any well known means, such as brine or electric refrigeration (not shown).

Immersion of the felt 10 in the caustic solution 18 is effected by the passage of the conveyor 12 and the felt 10 over guide roll 14 and under a second guide roll 31, both of which are adjustable to vary the period of immersion of the felt. Guide roll 14 is mounted in any convenient manner, as by suspending it from a cross bar (not shown), which is carried in a parallel take-up mechanism 33 that has adjusting screws 34 for varying its horizontal distance from guide roll 31 and thereby effecting an earlier or later immersion of the felt. Guide roll 31 is mounted in bearings 35, which are adjustable vertically by hand-wheels 36 to vary the depth to which the felt is immersed in tank 20. Guide rolls 16 and 17 are provided with adjusting hand- 100

wheels 37 and 38, respectively, for taking up or providing slack in the conveyor 12 as guide roll 31 is raised or lowered.

This immersion causes the felt to become impregnated with the caustic solution so that its fibers are swollen and their surfaces are slightly gelatinized.

The impregnated felt 10, supported on the conveyor 12, is passed between guide roll 15 and a second guide roll 39, the latter being adjustably mounted with respect to the former to permit the variation of the space between them by hand-wheels 40 and the exertion of any desired intense pressure. These rolls 10 squeeze the excess caustic solution from the felt 10, and form it into a rubber-like but very weak sheet, the expelled caustic flowing back 15 into tank 20.

A second wire screen conveyor 41, supported by a series of guide rolls 42, 43, 44, 45, and 46, mounted in a framework 47, and provided with tightening adjustments 48 and conveyor aligning adjustments 48', is mounted above the path of travel of the conveyor 12 and felt 10 to exert a predetermined and regulable pressure on the upper surface 25 of the felt to remove excess caustic solution.

The felt 10 supported on the conveyor 12, passes over a drum 49 that is perforated at 30 50 and heated by any desired means, such as steam supplied to a series of spray pipes 51. A suction hood 52 is preferably mounted on the framework 47 to remove the uncondensed steam. As the felt 10 and conveyor 12 35 reach the circumference of the drum 49, conveyor 41 is brought into contact with felt 10 and steam is injected through the latter, thus stopping the gelatinizing action of the cold caustic solution and, with the aid of 40 the pressure applied by the upper screen, molding the fibers into a compact felt 53, in situ.

As the felt 53 leaves the drum 49 it also leaves the conveyors 12 and 41 and is received 45 on a third wire screen conveyor 54, supported by a series of guide rolls 55, 56, 57, and 58, as well as by certain press rolls which will be described hereinafter.

Conveyor 54 carries the felt 53 over guide 50 rolls 55 and 56 and under a guide roll 61, the latter being submerged in an aqueous caustic bath 62 contained in a tank 63. This solution is of relatively high concentration and is maintained at a high temperature in 55 any suitable manner, as by gas or oil burners 64. This treatment reduces the swelling of the fibers and causes them to acquire more definite kinks and curls, accompanied by some shrinkage in the area of the felt.

The latter is now very strong and requires 60 only complete washing to free it from caustic, and for this purpose it passes through a series of rubber covered press rolls 65 which are independently adjustable at 66 to exert 65 any desired pressure and squeeze out the ex-

cess caustic. Showers of hot water, provided by spray jets 68, are directed upon the felt between each pair of press rolls, and the discharged water and caustic solution are collected in any suitable trough 70.

When the felt 53 leaves the last of these rolls it is entirely free from caustic and passes over any well known paper drying apparatus, such as the customary drying cans or steam heated rolls 71, or through a tenter 75 frame (not shown), and is wound up on a roll (not shown) or fed to other apparatus (not shown) which fits it for the special uses to which it is to be applied.

The apparatus is driven by any suitable 80 mechanism, such as a sprocket chain 72 which engages a sprocket wheel 73 on the axis of drum 49 and a series of sprocket wheels 74 on the driving shafts of the press rolls 65. These sprocket wheels are of any desired size, 85 and power is transmitted to sprocket wheel 73 from any suitable source (not shown). The power thus transmitted to the drum 49 is sufficient to create a friction drive for the various wire screen conveyors and to feed the 90 untreated felt 10 forwardly into contact with conveyor 12. I have found it desirable to provide scraper knives 75, 76, and 77 in the vicinity of roll 31, roll 39, and drum 49, respectively, to overcome any tendency of the 95 felt to follow the contour of these rotary members.

I have also found it desirable to provide the roll 31 with a series of staggered slots 78 and to cover it with a Monel metal screen 79 to break the vacuum which tends to form between it and the gelatinized fibers, although any equivalent means might be used.

Although the apparatus described herein is one I have found satisfactory for carrying 100 out my new process, I do not desire to be limited thereto because it forms no part of the present invention.

In the preferred form of my invention I use as the raw material a felt made from 110 kraft pulp in the manner indicated above, and pass it into a 10-11% aqueous sodium hydroxide solution at  $-5^{\circ}\text{C}$ . for a 5-second treatment, and for the second caustic treatment I use an 18% sodium hydroxide solution at  $100^{\circ}\text{ to }104^{\circ}\text{C}$ . for 5 seconds or longer.

If a sheet of unsized kraft, made from fibers that have not been curled and kinked, is used as the raw material a considerably longer time is required for impregnation 120 with the cold caustic solution.

If the starting material is a sheet made from 5-hour cooked cotton linters it should remain in the cold caustic solution 6 seconds, whereas if the sheet is made from 20-hour 125 cooked linters this time may be reduced to 3 seconds.

To produce a relatively stiff felt the time of impregnation in the cold caustic bath is increased, but if a relatively pliable felt is 130

desired the time of impregnation is decreased.

Consequently, according to the raw material used and the degree of pliability desired in the final product the time of impregnation with the cold caustic bath will vary from 1 to 30 seconds. If it is desired to give a longer treatment in the cold caustic solution the concentration of the latter may be reduced as low as 8%, and I have found that a range of from 8 to 15% concentration of sodium hydroxide is satisfactory for most purposes, although still higher concentrations may be used with sheets from certain fibers such as cotton, rag, or wood pulp fibers that have been cooked a long time, or artificial fibers, such as rayon.

The duration of the period in which pressure is exerted by the cold rolls may vary from 1 to 30 seconds, the upper limit being utilized for fibers that are not very reactive, such as slightly cooked wood fibers. The duration of the exertion of pressure on the perforated hot drum may also be varied, but usually corresponds to the time of pressing with the cold rolls.

The degree of pressure exerted by both the cold rolls and the hot drum may also be varied, a greater pressure being used for fibers that are only slightly reactive than for fibers that are very reactive.

The temperature of heating may be varied but the best results are obtained when steam is liberated on to the sheet with a pressure of at least 10 pounds. The best results are obtained when there is a very sudden change from the highly swollen to the final swollen state. This is accomplished by heating the sheet as quickly as possible. While this may be accomplished by merely passing the sheet over a heated roll, this is too slow for optimum results, hence it is preferable to augment the heating by injecting steam through the sheet.

The concentration of the hot caustic bath may be varied, using any concentration above 15%, but the 18% concentration is preferable because the quality of the product with this concentration is near the optimum, and because of economy in caustic.

The temperature of the hot caustic bath may be varied from 80° C. to the boiling temperature of the solution, but the best results are obtained when it is near the latter point, although with certain types of fibers a lower temperature is preferable to avoid appreciable degradation of the cellulose and weakening of the felt. In general I have found that the best temperature range is from 100° to 104° C.

The time of passage through the hot caustic bath may vary from 2 to 20 seconds, although the latter period causes appreciable deterioration of some types of fibers.

As an example of the increase in strength

in a sheet made by my process, I have found that a sheet made from kraft fibers and subjected to this treatment had its Elmendorf tear strength raised from 125-130 grams to 1200-1300 grams, and its tensile strength 70 in a 1" strip raised from 1400 to 18,000 grams. The strong kraft papers previously used showed a marked decrease in strength at the line of crease when such papers were creased, whereas felt made by this process 75 suffers no decrease in strength even after repeated creasing. Likewise, sheets made from kraft fibers subjected to my process are less stiff than kraft papers which have not been so treated and are free from the 80 decided "paper break" which is characteristic of the untreated kraft papers.

My treatment also produces a marked increase in the wet strength of kraft papers and felts subjected thereto, raising the wet 85 tensile strength from 2% of the dry strength to 20% or more of the dry strength.

I desire to have it understood that I may use sheets or mats of any cellulose fibers, such as kraft fibers, linters, sulfite treated 90 fibers, rope fibers, cotton fibers, including those reclaimed from tires, burlap fibers, or a mixture of two or more types of fibers, such as a mixture of kraft and rope fibers or kraft fibers and linters. In sheets made 95 from such mixed fibers the greater length of rope fibers adds strength to the finished product and the kraft fibers give an increased pliability. Linters that are free from very short fibers give a product of similar 100 strength to long rope fibers. Fibers from wood, in general, give products whose strength varies as the length of the fibers.

Although I have referred to the use of these fibers in the form of a sheet it will be 105 understood that they may be in the form of a mat, felt, or paper, and I prefer that they be unsized.

Where high density is required more reactive fibers should be used.

Although I have referred herein to caustic solutions and have mentioned caustic soda in particular, it will be understood that caustic potash or other fixed caustic alkali may be used.

I have found that it is desirable to heat the material while it is still under pressure to prevent the final product from becoming stiff and boardy.

Although the passage through the hot caustic bath can be omitted, I have also found that this increases the strength of the final product and improves the felting.

It will therefore be apparent that I have developed a process of making felted cellulose fiber products in which the fibers are held together in a sheet form by intermeshing, kinking and curling of the fibers instead of by the use of binding materials, such as 125 resins, glues, pyroxylin and rubber compo- 130

sitions; that my products are more pliable than products made by other processes; and that my products have a greatly increased wet strength, and an equal or greater dry strength than paper without being subject to the characteristic "paper break".

Felted cellulose fiber products made in accordance with my invention are useful for a wide variety of purposes, including a base for subjection to coating or impregnating processes with pyroxylin, rubber or other materials, as in the formation of fabrikoid or artificial leather; for impregnation in single or multiple layer thicknesses with solutions of phenolic condensation products; and without impregnation, as for felt hats, containers, shoe counters or box toes.

As many apparently widely different embodiments of this invention may be made without departing from the spirit and scope thereof, it is to be understood that I do not limit myself to the specific embodiments thereof except as defined in the appended patent claims.

25 I claim:

1. The process of making felted cellulose fiber products, which comprises gelatinizing continuous bands of cellulose fibers with caustic alkali, subjecting these gelatinized fibers to pressure and heat, and washing.

2. The process of making felted cellulose fiber products, which comprises treating cellulose fibers in sheet or mat form with caustic alkali to gelatinize these fibers without dispersing them, pressing while gelatinized, heating while maintaining pressure, and washing.

3. The process of claim 2, in which the caustic alkali solution is cold.

40 4. The process of claim 2, in which the fibers are subjected to a treatment with hot caustic alkali before the washing.

45 5. The process of making felted cellulose fiber products, which comprises treating cellulose fibers in sheet or mat form with an 8 to 15% solution of caustic alkali to gelatinize these fibers without dispersing them, pressing while gelatinized, heating while maintaining pressure, and washing.

50 6. The process of claim 5, in which the caustic alkali is maintained at a temperature below 5° C. and treatment with caustic alkali is continued for from 1 to 30 seconds.

55 7. The process of claim 5, in which the fibers are subjected to treatment with an 18% solution of hot caustic soda for from 2 to 20 seconds before the washing.

60 8. The process of claim 5, in which the caustic alkali is maintained at a temperature below 5° C. and treatment with this caustic alkali is continued for from 1 to 30 seconds, and in which there is a subsequent treatment with a hot 18% caustic alkali solution before washing.

65 9. The process of making a felted cellulose

fiber product, which comprises treating a felt made from kraft pulp, in which fibers have been curled and kinked, with a 10-11% caustic solution at a temperature of -5° C. for 5 seconds to gelatinize the fibers without dispersing the cellulose, pressing the gelatinized fibers, increasing the temperature while still maintaining the pressure, and washing to remove the caustic alkali.

70 10. The process of claim 9, in which the heating is facilitated by the application of steam under an initial pressure of at least 10 pounds.

75 11. The process of claim 9, in which the mat is passed through an 18% solution of sodium hydroxide at 100° to 104° C. for 5 seconds prior to the washing, to reduce the swelling of the fibers and facilitate their kinking and curling.

80 12. A strong flexible compressed felted non-woven cellulose fiber product comprising artificially an intensely curled and kinked fibers held together by gelatinization of the fibers.

85 13. A product comprising artificially curled and kinked cellulose fibers associated in a non-woven sheet form without other binder and having a wet tensile strength equal to at least 12% of its dry strength.

90 In testimony whereof, I affix my signature.

95 GEORGE L. SCHWARTZ.

100

105

110

115

120

125

130